

## UNITED STATES PATENT OFFICE

2,095,611

## INHIBITING THE CORROSION OF ALUMINUM

Homer E. McNutt, Rome, Ga., assignor to Tubize Chatillon Corporation

No Drawing. Application July 25, 1935,  
Serial No. 33,063

8 Claims. (Cl. 18—54)

This invention is concerned with inhibiting the corrosion of aluminum and aluminum alloys during exposure to solutions containing alkali metal sulfides. More particularly, the invention is concerned with the prevention of corrosion of aluminum carriers for artificial silk in desulphurizing processes. The invention also contemplates facilitating the desulphurization of viscose artificial silk filaments and the production of improved filaments of this character.

In the manufacture of artificial silk by the viscose process elemental sulphur and complex sulphur bodies are formed in the coagulation and regeneration steps and are entrapped within and upon the filaments. If these sulphur compounds are left associated with the filaments the final artificial silk product is of such poor appearance and quality as to be unsaleable. Consequently, it has been customary to remove these sulphur compounds by treating the filaments with a solution which acts as a solvent for such compounds.

In several of the heretofore customary processes for desulphurizing artificial silk, the material has been subjected to the action of desulphurizing solutions in the form of loose skeins. Thus, the freshly spun yarn is sometimes collected on a bobbin or in a bucket and then wound into loose skeins which are treated first to remove excess coagulant and then to remove sulphur. Another alternative is similar except that the yarn is dried after the coagulant is removed; the dried yarn being then wound into loose skeins which are desulphurized. The preparation and handling of the loose skeins in either of these ways is inconvenient and uneconomical. It is much more desirable to perform the desulphurizing operation while the yarn is retained on some type of carrier such as a bobbin. However, when the yarn is desulphurized on a carrier it is necessary to provide a carrier material which is not attacked by the desulphurizing solution.

Aluminum and aluminum alloys, on account of their lightness, strength and the ease with which they can be fabricated, may be used advantageously as materials for constructing bobbins, buckets and other carriers for artificial silk. The terms "aluminum" and "metallic aluminum" are hereinafter used to include aluminum and aluminum alloys.

Solutions of alkali metal sulfides, for example sodium sulfide, are efficient solvents for removing sulphur from viscose artificial silk. However, these sulfide solutions tend to corrode aluminum. In the heretofore customary art, attempts to use solutions of alkali metal sulfides in

contact with aluminum carriers have resulted in excessive corrosion of the aluminum with the formation of aluminum salts which are deleterious to the artificial silk. Furthermore, because of the tendency of such solutions to hydrolyze into sulphhydrates and the hydroxides of the alkali metals the solutions manifest a relatively high alkalinity. Probably because of this alkalinity, desulphurizing of artificial silk with solutions of alkali metal sulfides usually causes the silk filaments to swell and to become partly mercerized. The swelling and partial mercerization of the filaments appear to increase their resistance to penetration by the solvent for sulphur. In any event, when such swelling occurs the rate of sulphur removal is decreased both in the desulphurizing bath and in subsequent washing operations.

In other words, the use of aluminum carriers in the heretofore customary art of viscose artificial silk manufacture necessitated the preliminary washing and drying of the artificial silk and the removal of the yarn from the carrier in the form of loose skeins which were then desulphurized out of contact with aluminum.

Another practice of the heretofore customary art has been to desulphurize the viscose artificial silk on the carriers employing solvents which do not corrode aluminum to an appreciable degree. Such solvents, however, are usually less effective than solutions of alkali metal solvents and are frequently more expensive.

As a result of my investigations I have discovered that the presence of polysulfide sulphur in desulphurizing baths containing alkali metal sulfides serves a twofold purpose, in that it inhibits the corrosion of aluminum and at the same time inhibits the swelling of the artificial silk filaments. The presence of polysulfides in such desulphurizing baths, therefore, contributes the following advantages:

1. Corrosion of aluminum carriers may be substantially inhibited and almost completely prevented.
  2. Loss of reagents due to combination of the sulfides with aluminum is prevented.
  3. The presence of aluminum salts in the yarn (which has a deleterious effect upon the final product) is prevented; and
  4. Desulphurization of the yarn is accomplished more rapidly and with greater thoroughness.
- In order to obtain these fourfold advantages, I have found it desirable to maintain a relatively high concentration of polysulfide sulphur in the

desulphurizing solution. The molecular ratio between polysulfide sulphur and alkali metal monosulphide in the solution should be at least unity. When very concentrated solutions of alkali metal sulphides are used, I have found it advantageous to have slightly more than one molecule of polysulfide sulphur per molecule of alkali metal monosulphide in the solution.

A specific example of a satisfactory desulphurizing solution prepared in accordance with my invention may be conducive to a more thorough understanding of my invention. A solution containing approximately 2.4 grams per liter of sodium monosulphide is prepared by dissolving the commercial salt ( $Na_2S$ ) in water. To this solution flowers of sulphur equivalent to approximately 1.0 gram per liter of solution is added. The solution is then thoroughly agitated to accomplish a solution of the elemental sulphur as "polysulphide" sulphur. The solution is then ready for use.

The molecular ratio of elemental or "polysulphide" sulphur to sodium monosulphide in the above solution is:

$$\frac{1 \div 32}{2.4 \div 78.1} = 1.02$$

The elemental sulphur combines with the sodium monosulphide to form a polysulphide having a formula which may be exemplified as:



That is to say, additional sulphur is added to the monosulphide, the atomic proportions of the amount added being equal to the subscript  $x$ . As previously indicated,  $x$  should be approximately 1. The term "polysulphide sulphur" as used in this application refers to the sulphur " $S_x$ " which is added to the monosulphide molecule. The term "monosulphide sulphur" is used to indicate the normal sulphur content of alkali metal monosulphides, i. e. the "S" in " $Na_2S$ ".

The above described desulphurizing solution may be used either in a hot or in a cold condition, but very satisfactory results are obtained when the temperature of the solution during the desulphurizing treatment is maintained between 20 and 30° C. The solution is sucked or forced through the yarn for a period sufficiently long to dissolve and extract substantially all of the sulphur from the filaments. The yarn is then given a final wash with water. The yarn may then be treated directly or subjected to other customary subsequent treatments, such as bleaching.

The application of my invention is not limited to the protection of aluminum carriers alone. My invention also permits the use of other aluminum equipment such as tanks for handling alkali metal sulfide solutions used for desulphurizing.

Although the specific example given describes the addition of flowers of sulphur to the solution in order to produce the required polysulphide content, other sources of sulphur may be used conveniently. I have discovered that it is possible to produce satisfactory solutions by mixing fresh monosodium sulfide either as a solid or in the form of a concentrated solution with waste solutions withdrawn from the desulphurizing operation. By waste solutions, I mean those solutions which have dissolved such large quantities of sulphur from the filaments as to be no longer useful as solvents in their unchanged condition. Of course, when starting with fresh solutions it is desirable to add sulphur in the form

of elemental sulphur so that the correct ratio of polysulphide sulphur to sodium or potassium monosulphide will be obtained immediately. In a continuous process, however, I have found that the correct ratio of monosulphide to polysulphide sulphur can be maintained merely by adding fresh sodium monosulphide to the desulphurizing solution from time to time. The amount of solution which is lost by entrainment in the filaments is normally sufficient to bleed excess polysulphide sulphur from the bath. When high concentrations of alkali monosulphides are used (say 20 grams per liter), the entrainment loss of polysulphides may be too great to permit the maintenance of the correct ratio of monosulphide and polysulphide sulphur in the bath. In such case it may be necessary to add polysulphide sulphur (say in the form of flowers of sulphur) to the bath from time to time. By periodically analyzing the desulphurizing bath it may easily be determined whether or not to add alkali metal monosulphide and/or polysulphide to the bath.

Although my invention has been described with particular reference to the desulphurizing of viscose artificial silk in the presence of aluminum, it will also be clear that my invention is applicable to the desulphurization of viscose artificial silk when no aluminum is present, in that by maintaining the ratio of polysulphide to monosulphide sulphur in said solution at a sufficiently high concentration the swelling of the artificial silk filaments is prevented. Removal of the sulphur from the filaments is thus facilitated and accelerated.

My invention is applicable both to yarn which has been dried and to freshly spun filaments. The process may be applied successfully by immersing the artificial silk filaments in the solution, by forcing solutions through the yarn by vacuum or by pressure, and/or by placing yarn and solution in a suitable centrifuge.

I have found that when solutions containing approximately 2.5 grams per liter of sodium monosulphide and 1 gram per liter of polysulphide sulphur are used in the conventional pressure desulphurizing apparatus hours are necessary for a substantially complete removal of the sulphur from the freshly spun artificial silk. When more concentrated solutions are used, or when the temperature of the solution is increased above 30° C., the time of treatment may be reduced substantially.

I claim:

1. A process for inhibiting the corrosion of aluminum in the presence of solutions of alkali metal sulfides which comprises maintaining a ratio of polysulphide sulphur to monosulphide sulphur in said solutions of at least unity.

2. A process for inhibiting the corrosion of aluminum in the presence of solutions containing sodium sulfide which comprises maintaining the ratio of polysulphide sulphur to sodium monosulfide in said solutions at least at unity.

3. A process for inhibiting the corrosion of aluminum in the presence of a solution of alkali metal sulfide which comprises incorporating an alkali metal polysulfide into the solution.

4. In process for desulphurizing viscose artificial silk in the presence of metallic aluminum with a solution containing sodium sulfide the improvement which comprises increasing the sulphur content of the solution to form sodium polysulfide and maintaining the ratio of polysulphide sulphur to monosulfide sulphur in the solutions at not less than unity in order to inhibit corro-

sion of the aluminum and at the same time to prevent swelling of the viscose artificial silk.

5. In a process for desulphurizing viscose silk involving a preparation of a solution of an alkali metal sulfide and treatment of the viscose silk with the solution, the improvement which comprises incorporating in the solution an alkali metal polysulfide in predetermined amount prior to utilizing it for the treatment of silk.

0 6. In a process for desulphurizing viscose silk involving the preparation of a solution of an alkali metal sulfide and treatment of the viscose silk with the solution, the improvement which comprises incorporating in the solution alkali metal sulfide in predetermined amount by adding elemental sulphur to the solution prior to utilizing it for the treatment of silk.

5 7. In a process wherein artificial silk is desulphurized with a solution containing an alkali metal sulphide in the presence of metallic

aluminum, the improvement which comprises maintaining the ratio of the atoms of polysulphide sulphur to the atoms of monosulphide sulphur in the solution at a point not less than unity by adding to the solution an alkali metal polysulphide, thereby to prevent the corrosion of the aluminum and the swelling and partial mercerization of the artificial silk.

8. In a process wherein artificial silk is desulphurized with a solution containing an alkali metal sulphide in the presence of metallic aluminum, the improvement which comprises maintaining the ratio of the atoms of polysulphide sulphur to the atoms of monosulphide sulphur in the solution at a point not less than unity by adding to the solution elemental sulphur, thereby to prevent the corrosion of the aluminum and the swelling and partial mercerization of the artificial silk.

HOMER E. McNUTT. 20